

Sept. 14, 1926.

1,599,948

T. G. BLACKLOCK

TABLET FUEL

Filed Nov. 21, 1925



INVENTOR  
*Thomas G. Blacklock.*  
BY

*Harold D. Penney* ATTORNEY

Patented Sept. 14, 1926.

1,599,948

# UNITED STATES PATENT OFFICE.

THOMAS G. BLACKLOCK, OF PEEKSKILL, NEW YORK, ASSIGNOR TO MRS. THOMAS G. BLACKLOCK, OF NEW YORK, N. Y.

## TABLET FUEL.

Application filed November 21, 1925. Serial No. 70,574.

The present invention relates to compound fuel and the process of making the same, and especially to a compound fuel adapted for burning in its container or in a portable stove, and a principal object of the invention is to provide a fuel of this character which in manufactured commercial form is solid, moldable and safe and convenient to use, and which burns freely, completely and with a minimum of residue and substantially sootless, and which is well adapted for the various purposes where a ready to hand means for providing heat is required, such, as for toilet-making purposes, cooking of light meals or infant's food, picnics and the like.

A feature of the invention is the use of an absorbent combustible fibrous element having a capillary and absorbent capacity and having the novel function of acting as a means for absorbing the other combustible elements while they are in liquid form and containing and binding them when they are solidified, and also having a wick-like function during the combustion of the fuel for feeding and spreading the combustion area.

In the accompanying drawing is shown a perspective view of my new fuel, preferably in tablet, rectangular form, with one end cut away to show the cross section thereof.

In the drawing, A represents the section of cotton fibres, intermingled, within the body of the tablet, and B represents the outer hard surface of the body after cutting or molding to requisite sizes, said hard body being of a modified wax-like material containing within it, a volatile fuel element.

The fuel is made by melting one volume of wax such as paraffin to reduce the wax to a liquid and adding thereto from one-third to one-half volume of a combustible volatile fluid such as naphtha, benzine or gasoline of the ordinary commercial kind, stirring thor-

oughly the wax and fluid and while the mixture is still hot and liquid thoroughly saturating therewith a mass of combustible absorbent fibrous material having a capillary capacity, such as a mass of cotton fibre, and cooling the saturated mass after solidification, said mass, after such solidification being cut or molded into suitable sized tablet pieces, and packeted as desired.

In using the fuel it is desirable that it should be burned in a container, preferably of tin, designed for the purpose, not shown.

What I claim and desire to protect by Letters Patent is:

1. The fuel making process which consists in melting paraffin and adding to the melted paraffin gasoline, thoroughly stirring the melted wax and gasoline, thoroughly saturating with the mixture a mass of cotton fibre, and cooling the mass for solidification.

2. The fuel making process which consists in melting one volume of paraffin and adding to the melted paraffin from one-third to one-half volume of gasoline, thoroughly stirring the melted paraffin and gasoline, thoroughly saturating with the mixture a mass of cotton fibre, and cooling the mass for solidification.

3. As an article of manufacture and sale, a fuel consisting of paraffin, gasoline and cotton fibre.

4. As an article of manufacture, a fuel consisting of one volume of paraffin, approximately one-third of a volatile inflammable liquid fuel, and sufficient cotton to absorb said paraffin and fuel and to act as a wick therefor.

Signed at Poughkeepsie, in the county of Dutchess and State of New York, this 17th day of November A. D. 1925.

THOMAS G. BLACKLOCK.